

Nov. 19, 1935.

G. A. DORNIK

2,021,227

METHOD OF ISOLATING THE SEGREGATE IN INGOTS

Filed March 3, 1934

2 Sheets-Sheet 1

Fig. 4.



Fig. 3.



Fig. 2.



Fig. 1.



INVENTOR

George A. Dornin  
Byrnes, Stebbins & Blenko  
his attorneys

Nov. 19, 1935.

G. A. DORRIN

2,021,227

METHOD OF ISOLATING THE SEGREGATE IN INGOTS

Filed March 3, 1934

2 Sheets-Sheet 2

Fig. 7.



Fig. 5.



Fig. 6.



INVENTOR

George A. Dorrin  
Byrnes, Stebbins & Blanke  
his attorney

## UNITED STATES PATENT OFFICE

2,021,227

METHOD OF ISOLATING THE SEGREGATE  
IN INGOTS

George A. Dornin, Baltimore, Md.

Application March 3, 1934, Serial No. 713,849

10 Claims. (Cl. 29—160.4)

This invention relates to a method of salvaging the sound metal in ingots at their upper ends surrounding the pipe cavity and the segregated zone just under the pipe cavity.

5 As an ingot which has been poured gradually cools, the solidification of the metal results in shrinkage so that a cavity known as the piping forms centrally of the ingot and principally at its top. Moreover, a considerable proportion of 10 the impurities in the molten metal becomes segregated during the congealing of the ingot, the segregate being just below the piping.

The extent to which the piping and segregate extend downwardly into the ingot can be materially lessened by employing the procedure described and claimed in my copending application Serial No. 525,525, filed March 26, 1931. It is 15 obviously desirable to thus limit the depth to which the metal to be isolated extends, because 20 of the expense of removing unsound metal which is deeply embedded in the ingot. My invention is not limited, however, to the product of the particular process described in the above mentioned copending application.

25 It is the customary practice where the piping and segregate are to be eliminated from the ingot to cut off the entire top portion thereof; and the volume of the metal which is thus discarded and is only useful for remelting is relatively large 30 as compared with the volume of the total ingot.

Attempts have been made to displace the zone 35 of metal surrounding the central core or portion which it is desired to isolate and remove, by forcing a die axially of the ingot, as disclosed, for instance, in the patent to Ball No. 1,680,493. The process therein disclosed has such drawbacks that it has never gone into commercial use. The principle therein set forth is fundamentally defective 40 because the pressure of the die is effective for causing upward displacement of only the upper portion of the unsound metal in the segregate. It has been found impossible to force all of the 45 impurities upwardly into an isolated projecting portion, as shown in Figure 6 of the Ball patent, by his process.

In accordance with my invention, I produce 50 cleavage by artificial means between the core including the unsound metal to be isolated and the surrounding zone of metal. The gap or crevice produced between the core and the surrounding zone of metal permits the latter to be reshaped without appreciably changing the shape of the core; and by thus dividing the surrounding zone 55 of metal from the central core, I make it possible to displace this zone away from the core.

In this way, I so isolate the unsound metal that it is found in the end portion of the rolled steel or can be separated and discarded in any desired manner, as by cropping before the ingot is further treated.

5 In the accompanying drawings in which certain embodiments of my invention are illustrated:

Figure 1 is a vertical section through an ingot showing the pipe and underlying segregate;

Figure 2 is a vertical section through an ingot 10 in which cleavage has been produced artificially between the core, which includes the metal to be isolated, and the surrounding zone of good metal;

Figure 3 is a vertical section through an ingot 15 which has been treated as shown in Figure 2 and then upset to displace the surrounding zone away from the core;

Figure 4 is a view in side elevation of the ingot 20 of Figure 3 after reshaping to prepare the ingot for rolling;

Figures 5, 6, and 7 illustrate a modified embodiment of my invention; Figure 5 shows in vertical section an ingot into which a cleavage instrument has been driven between the core and the surrounding zone of metal; Figure 6 is a view 25 in central vertical section of this ingot after the surrounding zone has been displaced outwardly and axially of the ingot; and Figure 7 is a vertical sectional view of the same ingot after the zone has been upset to cause the core to project and stand alone.

In the ingot shown in Figure 1, the segregate 30 underlies the pipe cavity 12, the segregate extending downwardly in a cone shaped mass within surrounding metal 14 which is, for the most 35 part, sound and usable. If the customary procedure for eliminating the segregate 12 were followed, the ingot would be cropped approximately as indicated by the broken line A—A. This means that the sound metal 14 surrounding the 40 segregate is cropped off and used only for remelting. In order to recover this sound metal 14, I propose to produce cleavage between a central core 16, which includes the unsound metal 12 to be isolated, and the surrounding zone 45 14 of good metal. This cleavage permits the sound metal 14 to be displaced away from and below the core, permitting the latter to project so as not to contaminate the body of the ingot.

The principles of my invention have been 50 above stated broadly; and may be applied, with various modifications which will suggest themselves to those skilled in the art, in accordance with the requirements of the particular situation presented. In Figures 2, 3, and 4, I have 55

shown how these broad principles may be applied to the production of an ingot suitable for rolling. As shown in Figure 2, a cleavage instrument 18, wedge-shaped in radial cross section, is driven between the core 16 and the surrounding zone of metal 14. The preferred manner of producing such cleavage is to fit the cleavage instrument 18 with a separable cutter ring 19, in accordance with the teaching of my prior Patent No. 672,316, granted April 16, 1901. The ring prevents the punch from sticking in the metal and is inexpensive, so that it can be replaced, whereas the instrument 18 may be used again and again.

In this, the preferred embodiment of my invention, the instrument 18 is a cone shaped body, so that it will wedge the metal 14 outwardly during the punching operation. I have found that the angle of the wedge should be approximately 30°.

In order to facilitate this punching operation, the ingot may be acted upon while it is still at a sufficiently elevated temperature to be plastic, or after the ingot has been heated up to such temperature. In order to prevent upsetting of the lower end of the ingot, it may be confined within a containing die 21. A plug 21' in the bottom of this die is useful for pushing the ingot up out of the die, in case the ingot should stick. If the ingot has been heated up to the plastic temperature by concentrating the heat in the upper portion of the ingot (preferably about the upper half), leaving the lower portion sufficiently cool to resist deformation, the die 21 is unnecessary.

The surrounding zone of good metal has now been separated from the core 16; and the next step is to change the relative vertical locations of the surrounding zone of good metal and the core 16. This, as illustrated in Fig. 3, may be accomplished by an upsetting operation, using an upsetting die 26. The upsetting operation causes the zone of metal 14 to be pushed downwardly and become a part of the body of the ingot. Due to the plastic condition of the metal, a bulge 22 is formed at the top of the ingot, which is not objectionable if the ingot is to be further forged in producing the desired shapes. The core 16 projects from the upper end of the ingot; and may either be cropped at this time or be included in the metal discarded after subsequent forging operations. The steps of dividing the core from the surrounding zone of metal and then changing the relative vertical locations of the surrounding zone of metal and the core containing the segregate leave the core in such position relative to the ingot that it no longer requires cropping of sound metal along with the unsound core.

For rolling in a rolling mill, the shape of the ingot as shown in Fig. 3 is unwieldy; and a further step of forging is in that case preferably added to reduce the section of the bulging portion 22 of the ingot so that it may be suitable for rolling. The ingot shown in Fig. 4 has been thus forged to reduced the enlarged portion 22 to substantially its original section.

In accordance with the modification of my invention illustrated in Figs. 5, 6, and 7, a cleavage instrument 23 is driven down into the top of the ingot to divide the core 16 including the unsound metal to be isolated from the surrounding zone of metal 24. Following this step, an expanding die 26 is pushed downwardly into the cleavage thus produced. The face 27 of the die 26 which engages the surrounding zone of metal

should be disposed at an angle to the horizontal so as to deflect the surrounding zone of metal outwardly. The next step is to displace the surrounding zone of metal into the body of the ingot as illustrated in Fig. 7. Obviously, if an ingot suitable for rolling is desired, the ingot shown in Fig. 7 may be further forged to suitable shape for rolling as above described in connection with Fig. 4.

In both embodiments of the invention, the surrounding zone of metal is divided from the core including the unsound metal to be isolated. In an ingot poured in a mold of generally round cross-section, such as octagon and dodecagon molds, the segregate is substantially cone-shaped, and the cleavage instrument should correspondingly have a substantially circular cutting edge. With molds whose cross-section is elongated, such as rectangular molds, the ingot will have a segregate whose shape is similar to that of the mold with the corners rounded off. The cleavage instrument will, therefore, have a cutting edge which, instead of being circular, will correspond substantially to the shape of the segregate; and may for instance be substantially elliptical, or a circle flattened on two sides. The opening in the die 26 and in the upsetting die 20 will be sufficiently larger than the core 16 so as not to touch or bind on the core during the expanding or upsetting operations.

The purpose of deflecting the surrounding zone of metal outwardly is to better prepare it for the upsetting operation. When a mass of plastic metal is upset, there is a bulge formed; and if the surrounding zone of metal were merely divided from the central core as shown in Fig. 5, the upsetting operation would cause this zone of metal to overlap back on the cylindrical core during the upsetting operation, and might bring about a welding of the two together which would defeat the purpose of the first step of the process. The deflection of the surrounding zone is sufficient if the angle of the wedge is substantially 30° to the vertical. The deflection is accomplished in the first embodiment in the same step in which the cleavage is effected. In the second embodiment, this is accomplished in two steps.

In the specification and claims I have used the term "artificial cleavage" to distinguish the predetermined cleavage effected in accordance with my teaching from separation or cleavage which may occur as cracks or the like due to shrinkage or other natural causes.

Starting with an ingot whose cooling has been properly controlled, the weight of the isolated segregated metal in the cylindrical core 16 need not be over 2% of the weight of the ingot. There are other inescapable losses, such as the scale loss incurred in heating the ingots, and the bottom prop; but it is possible to limit the total losses to from 5 to 7%, leaving 93 to 95% of good product. It is considered good practice in producing big-end-up sink-head ingots to obtain 80 to 82% good product. It will be apparent, therefore, that the expense incurred in treating an ingot in accordance with my invention is small compared with the saving which can be effected.

While I have illustrated and described certain embodiments which my invention may assume, and certain equipment which may be employed in carrying out the same, it will be understood that the practice of the invention is not dependent upon the particular equipment referred to and may be otherwise embodied and practiced within the scope of the following claims.

I claim:

1. In a method of isolating unsound metal of an ingot, the steps consisting of making a gap or crevice between a core including the unsound metal to be isolated and the surrounding zone of metal, without substantial displacement of the core axially of the ingot to divide said core from said zone, and displacing said zone away from said core.
  2. In a method of isolating unsound metal of an ingot, the steps consisting of making an incision between a core including the unsound metal to be isolated and a surrounding zone of metal, and thereafter upsetting said zone to displace the good metal away from said core.
  3. In a method of isolating unsound metal of an ingot, the steps consisting of wedging a surrounding zone of metal away from a central core including the unsound metal to be isolated, and displacing said zone axially of the ingot.
  4. In a method of isolating unsound metal of an ingot, the steps consisting of dividing a surrounding zone of metal from a central core including the unsound metal to be isolated, and displacing said zone outwardly and axially of the ingot.
  5. In a method of isolating unsound metal of an ingot, the steps consisting of artificially dividing the unsound metal of an ingot from the sound metal that surrounds it, and then changing the relative vertical locations of this good metal and unsound metal by upsetting the good metal only.
  6. In the method of isolating unsound metal of an ingot, the steps consisting of artificially dividing the unsound metal of an ingot from the sound metal that surrounds it, then changing the
- relative vertical locations of this good metal and unsound metal by upsetting the good metal only, and then forging the enlarged upset end of the ingot substantially back to its original size.
7. In a method of isolating unsound metal of an ingot, the steps consisting of dividing a surrounding zone of metal from a central core including the unsound metal to be isolated, upsetting said zone axially of the ingot and then forging the upset portion of the ingot to displace the upset metal inwardly.
  8. In a method of isolating unsound metal of an ingot, the steps consisting of wedging a surrounding zone of metal away from a central core including the unsound metal to be isolated, upsetting said zone and then forging the upset portion of the ingot to reduce said portion substantially to its original section.
  9. In a method of isolating unsound metal of an ingot, the steps consisting of wedging a surrounding zone of metal away from a central core including the unsound metal to be isolated, the angle of the wedge being not less than about 30°, and changing the relative vertical locations of the surrounding zone and central core by upsetting the surrounding zone of metal only.
  10. In a method of isolating unsound metal of an ingot, the steps consisting of dividing a surrounding zone of metal from a central core including the unsound metal to be isolated, deflecting the surrounding zone of metal away from the core by an included angle of at least about 30°, and displacing said surrounding zone axially of the ingot.

GEORGE A. DORNIN. 35

### CERTIFICATE OF CORRECTION.

Patent No. 2,021,227.

November 19, 1935.

GEORGE A. DORNIN.

It is hereby certified that error appears in the printed specification of the above numbered patent requiring correction as follows: Page 3, first column, line 8, claim 1, after "and" insert thereafter; and that the said Letters Patent should be read with this correction therein that the same may conform to the record of the case in the Patent Office.

Signed and sealed this 7th day of January, A. D. 1936.

(Seal)

Leslie Frazer  
Acting Commissioner of Patents.

I claim:

1. In a method of isolating unsound metal of an ingot, the steps consisting of making a gap or crevice between a core including the unsound metal to be isolated and the surrounding zone of metal, without substantial displacement of the core axially of the ingot to divide said core from said zone, and displacing said zone away from said core.
  2. In a method of isolating unsound metal of an ingot, the steps consisting of making an incision between a core including the unsound metal to be isolated and a surrounding zone of metal, and thereafter upsetting said zone to displace the good metal away from said core.
  3. In a method of isolating unsound metal of an ingot, the steps consisting of wedging a surrounding zone of metal away from a central core including the unsound metal to be isolated, and displacing said zone axially of the ingot.
  4. In a method of isolating unsound metal of an ingot, the steps consisting of dividing a surrounding zone of metal from a central core including the unsound metal to be isolated, and displacing said zone outwardly and axially of the ingot.
  5. In a method of isolating unsound metal of an ingot, the steps consisting of artificially dividing the unsound metal of an ingot from the sound metal that surrounds it, and then changing the relative vertical locations of this good metal and unsound metal by upsetting the good metal only.
  6. In the method of isolating unsound metal of an ingot, the steps consisting of artificially dividing the unsound metal of an ingot from the sound metal that surrounds it, then changing the
- relative vertical locations of this good metal and unsound metal by upsetting the good metal only, and then forging the enlarged upset end of the ingot substantially back to its original size.
7. In a method of isolating unsound metal of an ingot, the steps consisting of dividing a surrounding zone of metal from a central core including the unsound metal to be isolated, upsetting said zone axially of the ingot and then forging the upset portion of the ingot to displace the upset metal inwardly.
  8. In a method of isolating unsound metal of an ingot, the steps consisting of wedging a surrounding zone of metal away from a central core including the unsound metal to be isolated, upsetting said zone and then forging the upset portion of the ingot to reduce said portion substantially to its original section.
  9. In a method of isolating unsound metal of an ingot, the steps consisting of wedging a surrounding zone of metal away from a central core including the unsound metal to be isolated, the angle of the wedge being not less than about 30°, and changing the relative vertical locations of the surrounding zone and central core by upsetting the surrounding zone of metal only.
  10. In a method of isolating unsound metal of an ingot, the steps consisting of dividing a surrounding zone of metal from a central core including the unsound metal to be isolated, deflecting the surrounding zone of metal away from the core by an included angle of at least about 30°, and displacing said surrounding zone axially of the ingot.

GEORGE A. DORNIN. 35

### CERTIFICATE OF CORRECTION.

Patent No. 2,021,227.

November 19, 1935.

GEORGE A. DORNIN.

It is hereby certified that error appears in the printed specification of the above numbered patent requiring correction as follows: Page 3, first column, line 8, claim 1, after "and" insert thereafter; and that the said Letters Patent should be read with this correction therein that the same may conform to the record of the case in the Patent Office.

Signed and sealed this 7th day of January, A. D. 1936.

(Seal)

Leslie Frazer  
Acting Commissioner of Patents.